

## UNITED STATES PATENT OFFICE.

WILLIAM H. ALLEN, OF DETROIT, MICHIGAN.

## PICKLING-BATH.

1,321,182.

Specification of Letters Patent. Patented Nov. 11, 1919.

No Drawing.

Application filed May 10, 1917. Serial No. 167,656.

*To all whom it may concern:*

Be it known that I, WILLIAM H. ALLEN, a citizen of the United States, and residing at Detroit, in the county of Wayne and State of Michigan, have invented a new and Improved Pickling-Bath, of which the following is a specification.

This invention relates to processes for the cleaning of surfaces of iron or steel by means of pickling baths, and its object is to so change the otherwise slowly soluble scales and particles of the higher oxids that they may be quickly absorbed by the pickling solution and therefore offer no continued obstruction to the action of the bath on the metal beneath such coverings.

This process consists in changing the patches of scale, rust and other forms of higher oxids on the surfaces of articles of iron and steel being cleaned, by means of a solution of a strong reducing agent, to a ferrous or lower condition when they become readily soluble in the solution of the inorganic acid used to clean the articles, the reducing agent and the acid preferably being in the same solution, although they may be in separate solutions.

Patches of scale or rust often occur on the surfaces of articles of iron or steel that are to be cleaned by pickling in an acid bath and because these patches of higher oxid are much more slowly dissolved by the acid than the metal itself, the surfaces that are being pickled are irregularly attacked by the acid in the bath, resulting in the pitting of the surfaces that are being cleaned.

The use of a strong reducing agent in the bath materially equalizes the action of the acid by first rapidly changing the ferric condition of the oxids and scale to the ferrous condition, after which complete absorption by the bath is very rapid.

The ordinary pickling bath is usually a solution of an inorganic reducing acid, such as sulfuric, hydrochloric or phosphoric acid. A ten per cent. solution of sulfuric acid is probably more common than any other. The action of this bath on the patches of scale usually found on rolled

sheet metal is slow compared to its action on the bare metal and the sheet metal therefore often comes out of the pickling bath very uneven in thickness. By adding sulfurous acid to this bath to the solution of sulfuric, hydrochloric or phosphoric acid, either by blowing sulfur dioxide through it or by adding a sulfite or bisulfite or hyposulfite of sodium, which will be decomposed by the acid, a pickle is obtained that will act substantially equally on the entire surface being treated. The effective sulfurous acid should equal about one fifth of the effective sulfuric acid but an excess of the reducing agent is not objectionable. The reducing agent rapidly changes the iron oxid in the ferric condition to ferrous oxid, which is quickly dissolved by the sulfuric acid.

Phosphorous acid, hydrogen sulfide and sulfides of iron or sodium may be substituted for the sulfurous acid if desired. Phosphides of iron or zinc in a sulfuric acid solution liberate phosphine which is also a valuable reducing agent. Solutions of acid sulfates and acid phosphates may be employed in place of the solutions of the acids.

After the metal has been cleaned it may be immediately rinsed in a dilute solution of a proper reducing agent and then dried, or otherwise treated to prevent the formation of ferric iron.

I claim:—

1. The process of cleaning surfaces of iron and steel spotted or covered with scale or rust which consists in treating the same with sulfurous acid in a solution of sulfuric acid.

2. The process of cleaning surfaces of iron and steel having patches of higher oxids of iron on the metal which consists in immersing the same in a bath wherein the higher oxids will be reduced by sulfurous acid and then absorbed by sulfuric acid which slowly dissolves the metal, removing the articles from the bath and treating them to prevent rusting.

WILLIAM H. ALLEN.